

**METHOD OF PROVIDING FERROUS ARTICLES  
WITH PHOSPHATE COATINGS AND COMPOSI-  
TIONS THEREFOR**

John A. Henricks, Logansport, Ind.  
(742 N. Oak Park Ave., Oak Park, Ill.)

No Drawing. Filed Jan. 22, 1957, Ser. No. 635,130

2 Claims. (Cl. 148—6.15)

This invention relates to the formation of integral phosphate coatings on metallic surfaces. More particularly, it relates to phosphate coating baths for forming on metallic surfaces improved phosphate coatings which are characterized by having a micro-crystalline or amorphous-like structure.

The almost universal practice in the automotive and appliance industries is to form a zinc, iron, or manganese phosphate coating on the surfaces of ferrous metals which are to be painted or enameled, drawn, adhered to or otherwise fabricated. The phosphate coating baths in general use form an integral phosphate coating which consists of many relatively large, elongated crystals. In contrast, the phosphate coating baths of the present invention form an integral phosphate coating which consists of a multiplicity of fine, interlaced microcrystalline grains as will be hereinafter described.

Phosphate coating baths are prepared by dissolving phosphoric acid and/or dihydrogen phosphate salt mixtures in water together with oxidizers and other additives to form a concentrate and then diluting the concentrate with water to form a coating bath which is nearly saturated with the phosphate salt. The baths are heated to temperatures of from 110° to 200° F. and the work is dipped in the bath or is sprayed with the bath so as to form a phosphate coating on it.

The bath will coat only so long as it is maintained within certain ranges of acidity, phosphate content, free acid content, etc. or, in other words, is in balance. The conventional means of analyzing baths to keep them in balance is to determine the specific gravity, free acid and total acid. The free acid is determined by titrating a 10 ml. sample of the solution to a bromphenol blue end point with N/10 sodium hydroxide. The total acid, or points, is determined by titrating a 10 ml. sample of the solution to a phenol phthalein end-point with N/10 sodium hydroxide.

One way in which phosphate coating baths are made up is to prepare a dry mixture of suitable chemicals and pour the mixture into a tank of water to form a coating bath. However, difficulty is encountered in storing these dry compositions in commercially used containers due to the deliquescent nature of the chemicals, particularly zinc nitrate and calcium chloride, which leads to the formation of a mushy, partially fused mass inside the container.

In the fabrication of metals where a high gloss finish is desirable a fine crystal or amorphous phosphate coating has distinct advantages. The preparation of such a phosphate coating has been an exceedingly difficult problem and in general the industry has had to accept relatively large crystal phosphate coatings where phosphate flakes off the metal when it is bent or flexed.

One object of the present invention is to provide phosphate coating baths and methods of compounding them so as to form integral microcrystalline or amorphous phosphate coatings on metallic surfaces which will permit

excessive bending or flexing of the phosphated metal without the flaking off of the coating.

Another object of the present invention is to provide a powder make-up composition for phosphate coating baths which remains relatively dry and free flowing even though stored for long periods of time.

Another object of the present invention is to provide phosphate coating baths which form integral microcrystalline phosphate coatings on metallic surfaces and which are readily operable in production in that they coat within a reasonable time, can be kept in balance without difficulty and are otherwise easy to handle.

Other objects and advantages will become apparent from the following description of the present invention.

15 I have found that when certain metallic ions such as the calcium ion and an accelerating agent such, for example, as a nitrate or nitrite are added in regulated quantities to aqueous acidic zinc, iron, or manganese phosphate coating baths, the baths form an improved microcrystalline or amorphous phosphate coating. I have further found that, in order to maintain an operable bath, the metallic ions, accelerating agent, and phosphate ions have to be present in certain critical ratios.

20 The compositions prepared in accordance with this invention are preferably based upon nitrate depolarized formulations prepared from phosphoric acid or highly soluble phosphates and highly soluble salts of zinc in proportions equivalent to an orthophosphate of zinc. Since the ingredients are all readily soluble, the hydrolysis and 25 sludge forming defects of the conventional dihydrogen phosphate compositions are avoided and, moreover, the ratio of zinc salts to phosphoric acid is not limited by considerations of solubility. Consequently, nearly any 30 degree of zinc supersaturation is possible up to 10 mols of zinc salt to each mol of phosphoric acid, and in low zinc content formulations, the ratio may be as low as one unit of zinc salts to four units of phosphoric acid. In the 35 simplest of such formulations, the zinc is all incorporated as zinc nitrate but the desired zinc saturation may also be 40 secured by providing at least a part of the zinc in the form of zinc chloride with the range of balance being from 10 units of zinc nitrate to 1 unit of zinc chloride, in a high nitrate formulation, to 1 unit of zinc nitrate to 3 units of zinc chloride, in low nitrate formulations. 45 The chloride acts to improve the non-sludging characteristics of the bath and also effects coating at a faster rate than baths which have all of the zinc in the form of the nitrate. Ammonium yielding substances may also be incorporated, as for example, by employing ammonium phosphate directly in the preparation of the 50 composition or by utilizing other substances therein which will facilitate the production of the ammonium radical.

55 In the above ratios and other critical values which may be found herein in which zinc is conveniently used as the principal coating ion, iron and manganese may be substituted for the zinc when the former ions are used as the principal coating cation. Also, the principal coating cation may be a mixture of one or more of the above ions.

60 The desired calcium content may be obtained by adding calcium to the solution, or to a concentrated makeup material, in a variety of its available forms including calcium oxide, calcium hydroxide, calcium nitrate, calcium chloride, calcium hydrogen phosphate, calcium dihydrogen phosphate, etc. Broadly, the calcium may be introduced in the form of any salt which is soluble in the solution and the anion portion of which is not detrimental to the coating-forming ability of the solution. The preferred calcium to zinc ratio is from about 0.5 to 4.5.

65 While the calcium ion is preferred as the modifier for

producing the amorphous coatings of the present invention, an ion from a member of the group consisting of lithium, beryllium, magnesium, calcium, strontium, cadmium and barium may be used to obtain a substantial portion of the benefits obtainable with the calcium ion. These ions are preferably added in the form of their nitrate salt although other soluble salts may also be used.

In order to coat within a reasonable time and overcome the positioning effect of the modifier, the coating baths of the present invention may contain nitrogen oxide depolarizer in the form of conventionally employed accelerating or oxidizing agents such as a hydrogen or alkali metal nitrate, nitrite or chlorate, nitrosyl chloride or the like. The preferred oxidizing agent is one containing nitrogen oxide, i.e. a nitrogen oxide depolarizer such as a nitrate or nitrite.

Taking nitrate as the most representative member of the class of nitrogen oxide depolarizer or oxidizing agents that may be used, the ratio by weight of nitrate to phosphate,  $(NO_3/PO_4)$  may extend from .16 to about 10.0 when the proportions and ratios of calcium and zinc above given are observed and best results are obtained when the ratio is about 1 to 4. A suitable amount of nitrate is readily determined by adding it to a coating bath until satisfactory coating action is obtained. The actual amount of nitrate in the preferred compositions of the present invention generally works out to be about 0.5 to 48 grams per liter. Other oxidizing agents may be used instead of nitrate, but when used should be employed in amounts which will produce approximately equivalent amounts of oxidizing or acceleration of coating formation. When chlorate is used, the ratio of  $ClO_3$  to  $PO_4$  is preferably from about .07 to about 1.8; for nitrite, the ratio of  $NO_2$  to  $PO_4$  may extend from about 0.003 to about 0.1 and is preferably about 0.015 to .04; for hydrogen peroxide, the preferred ratio may extend from about .003 to 0.01 and for dinitrobenzene sulfonate the preferred ratio may extend from about 0.15 to 1.0. Other oxidizing agents such as bromates, iodates, pteric acid, t-butyl hydroperoxide, quinones, etc. may be used, if desired, in quantities which produce an effect on the coating formation equivalent to that which is produced by the above specified range for nitrate. Mixtures of oxidizing agents may be used, if desired, with the desired quantity being that which produces an effect on the coating equal to the effect obtained from the use of nitrate in quantities as previously stated.

When the oxidizing agent is one other than nitrate it is to be understood that it may be necessary to incorporate a quantity of an additional anion that is substantially innocuous to the coating or coating forming ability of the solution, such as chloride, to effectively maintain the ionic balance of the solution. Instead of supplementing the need for anions with chloride or other innocuous anion it may be desirable to introduce all or part of the calcium as calcium nitrate.

While oxidizing agents are generally employed as the accelerator, reducing agents such as sodium sulfite, hydrazine salts or solution, chloral hydrate or the like may also be used as the accelerating agents.

The resulting acceleration of the coating composition is such that complete coating of a metal surface can be effected in from 3 to 5 minutes with an immersion bath at a temperature in the order of 200° F. in contrast to the 30 minutes required for coating by a conventional zinc dihydrogen phosphate bath and 10 minutes when conventional coating baths are modified by additions of zinc or sodium nitrate. Moreover, the coating produced from baths of the dihydrogen phosphate type, or those modified by the addition of zinc or sodium nitrate, are crystalline in nature while the coatings produced from baths to which a calcium salt or other modifier salt has been added, in at least the minimum quantities herein-after specified, have a smooth texture exhibiting no visible crystal structure even when examined under magnifica-

tion of 100 diameters. Furthermore, the chemical analysis of these amorphous-type coatings, when zinc is the principal coating cation used, reveals that they are mixed phosphates with the metal of the recited group occurring

6 therein in the ratio of about  $\frac{1}{2}$  mol thereof to each mol of zinc; the composition of the coating when lithium is used, for example, being  $Zn_2Li(PO_4)_2$ . Electronic diffraction analyses of the coatings indicates they are apatitic in nature. Thus, such analysis of a coating produced on

10 low carbon steel by a bath prepared in accordance with this invention and containing calcium and chlorine showed the coating to be microcrystalline or amorphous-like and have a diffraction pattern of an apatite with the pattern slightly distorted by the presence of zinc and iron.

15 A zinc phosphate coating bath is preferred in accordance with the present invention since it appears that there is a co-deposit of calcium or other modifier cation and that the phosphate coating actually contains the calcium or other ion in addition to zinc.

20 The concentration of zinc in the diluted bath of the present invention is preferably in the range of about 1 to 4 grams per liter with the best results being obtained at a concentration of about 2.0 to 3.5 grams/liter. As is well known in the art, however, zinc phosphate coating baths may be made up that contain as low as concentration as  $\frac{1}{2}$  gram/liter and as high a concentration as 10 up to even 15 grams per liter.

25 The amount of phosphate used is enough so that ratio of zinc to phosphate is preferably from about 6.8 to 1 to about .17 to 1, with the best results being obtained with a ratio of about 3 to 1 to about 0.5 to 1.

30 The amount of phosphate in the preferred baths of the present invention works out to be generally from about .15 to 24 grams/liter with best results obtained with from about 0.5 to 12 grams/liter using the preferred amounts of zinc as previously discussed.

35 In accordance with the present invention, the amount of calcium present varies with the amount of zinc present. The preferred amount is, as previously stated, enough to 40 keep the ratio of calcium ion to zinc ion in the range of about .5 to 4.5 by weight. There should be at least enough of the modifying cation (calcium) to maintain a ratio of it to the principal coating cation (zinc) of at least about .16 to 1 in order to obtain enough inhibiting action on the deposit of large crystals to obtain a satisfactory coating in accordance with the present invention. On the other hand, amounts of modifying cation which make a ratio of calcium to zinc larger than 10 to 1 prevent a satisfactory coating action. For most applications, 45 the amount of calcium or other modifying cation in the diluted bath is preferably about .5 to 18 grams/liter as hereinafter described as "the threshold value" of the salt of modifying cation. When a ferrous metal surface has been thoroughly etched by acid pickling or the like, more of the modifying cation is required than when the surface is not as clean as, for example, when a surface of ferrous metal stock is treated that has been merely wiped with a solvent such as carbon tetrachloride.

50 Other salts may also be used in accordance with the present invention to give manganese or iron phosphate coatings. Manganese phosphate coatings are similar to zinc phosphate coatings in weight and composition and are as satisfactory except that they are more expensive and so not generally employed. Iron phosphate coatings 55 are lighter in weight and are a mixture of iron oxides and iron phosphate. They are the least expensive of any coating and also the least satisfactory for many purposes although they do have special uses. In addition to forming an integral phosphate coating on iron and steel ferrous surfaces, baths of the present invention may also be used to coat zinc, aluminum, and many other metallic surfaces.

60 As mentioned above, the addition of a soluble salt of calcium, or other amorphous coating producing cation, to one of the nitrate or nitrogen oxide depolarized formula-

tions of the type mentioned, acts to accelerate the coating rate and inhibit crystalline growth, the extent of crystalline inhibition depending upon the amount of additive metal employed.

There appears to be a minimum amount of a modifier such as calcium which must be added to the bath in order to substantially eliminate the crystalline structure. This amount may be defined as the "threshold value" of the modifier and these values as determined for commercial grade materials on clean metal panels employed in a broken-in, 25 point bath, compounded as in Example I below, containing approximately 3.2 grams per liter of zinc and approximately 0.5 gram per liter of iron, are substantially as follows:

| Chemical                                                                       | Formula Weight | Concentration Required, grams/liter | Mol Percent |
|--------------------------------------------------------------------------------|----------------|-------------------------------------|-------------|
| Lithium Nitrate.....                                                           | 69             | 12.3                                | 18          |
| Beryllium Nitrate.....                                                         | 187            | 9.3                                 | 5           |
| Magnesium Nitrate.....                                                         | 256            | 25.6                                | 10          |
| Calcium Nitrate Ca-<br>(NO <sub>3</sub> ) <sub>2</sub> ·4H <sub>2</sub> O..... | 235            | 7.8                                 | 3           |
| Strontium Nitrate.....                                                         | 212            | 14.1                                | 6           |
| Cadmium Nitrate.....                                                           | 308            | 30.8                                | 10          |
| Barium Nitrate.....                                                            | 261            | 5.2                                 | 2           |

#### Example I

A 20 to 30 point bath zinc dihydrogen phosphate is prepared by diluting, to a 2 to 3% by weight solution, a concentrate containing:

| Chemical                                                                          | Units, Formula Weight×No. of Mols | Composition, Percent by Weight |
|-----------------------------------------------------------------------------------|-----------------------------------|--------------------------------|
| Phosphoric Acid H <sub>3</sub> PO <sub>4</sub> .....                              | 98×0.2                            | 19.6                           |
| Mono-Ammonium Phosphate<br>(NH <sub>4</sub> ) <sub>2</sub> HPO <sub>4</sub> ..... | 115×0.2                           | 23.0                           |
| Zinc Chloride ZnCl <sub>2</sub> .....                                             | 136×0.1                           | 13.6                           |
| Zinc Nitrate Zn (NO <sub>3</sub> ) <sub>2</sub> .....                             | 189×0.1                           | 18.9                           |
| Water added to dissolve salts.....                                                |                                   | 24.9                           |
|                                                                                   |                                   | 100.0                          |

This solution is then broken in and balanced to provide a 20 to 30 point bath by a trial load of ferrous articles thereby providing iron ions in the bath. To the balanced and broken-in bath there is added a nitrate of lithium, beryllium, magnesium, calcium, strontium, cadmium or barium in quantities approaching equimolarity so as to be within the threshold values given above with the zinc. The bath is then ready for use and will be found to provide a tight, microcrystalline coating.

The above specified threshold values are based upon technical or commercial grade nitrates which contain traces of other metals as impurities. For example, the calcium nitrate was found to have at least traces of strontium and magnesium. Lithium nitrate was found to have at least traces of aluminum, tin and strontium; calcium nitrate contained traces of strontium, fluorine, iron, aluminum and magnesium; and barium nitrate contained traces of cerium, titanium and calcium. These trade impurities have also been detected in the coatings by spectographic analysis and they evidently have an auxiliary or synergist action in inhibiting crystalline growth since the threshold concentrations of the modifier are materially less when employing commercial grades of the modifier material than when chemically pure grades of the modifiers are employed.

While the above listed threshold values have been given for baths containing 3.2 grams per liter of zinc, substantially the same values are valid for baths ranging in zinc content from 1 to 4 grams per liter.

The required amount of the modifying metal salt to produce the amorphous coating may be reduced by the additional smoothing effect of minor amounts of other materials. For example, the elements known as the amphoteric metals and which furnish the central coordi-

nating atom in the formation of heteropoly acids, as is discussed in "Inorganic Chemistry" by Fritz Ephraim, 4th edition, pages 500 to 509, may be so used. Of such elements, which include phosphorous, arsenic, antimony, 5 boron, thorium, silicon, tin, cerium, titanium, cobalt, zirconium, iron, vanadium, aluminum, copper, manganese, chromium, iodine and germanium, those are preferred which do not form an immersion deposit on iron or do not tend to poison the bath by preventing depositing of zinc phosphate. Besides iron, the safest auxiliary modifying agents are the soluble salts of cerium, zirconium, vanadium and titanium, these being utilized in concentrations of less than 1 gram per liter of the bath. In addition, trace amounts of antimony and arsenic, 10 which form immersion coatings of the iron but do not accelerate electrolytic corrosion of the iron, may be employed.

Although minor amounts of the additive substances mentioned may be employed for securing synergistic action in obtaining non-crystalline zinc phosphate coatings, 15 it is presently preferred to simply employ commercial grade nitrates or other soluble salts of lithium, beryllium, magnesium, calcium, strontium, cadmium or barium thereby taking advantage of the trace impurities therein.

Likewise, the iron, acquired in normal operation of 20 commercial phosphating baths when coating ferrous surfaces, assists in the formation of the desired coating although the concentration of this iron should not exceed 1 gram per liter.

The iron concentration does not materially increase 25 during normal working of the bath with ferrous articles probably because of the oxidizing action caused by the air and by the interaction of the nitrate and chloride of the zinc salts. However, in heavily worked baths, such

as spray installations for ferrous articles where the iron concentration tends to increase, such increase may be controlled by the periodic addition of barium or sodium nitrite, or calcium hypochlorite, in amounts of less than 30 1 gram per liter. It should also be mentioned that the aforementioned oxidation is solely for the purpose of acceleration and reduction of ferrous iron to thereby maintain a smooth amorphous coating through avoiding the deposit of coarse iron phosphate crystals. There is no need to effect oxidization of hydrogen in baths compounded in accordance with this invention since the high content of nitrate or its equivalent thereof provides adequate depolarization.

Although the addition of nitrates of lithium, beryllium, 35 magnesium, calcium, strontium, cadmium or barium to a zinc orthophosphate composition has been heretofore described specifically with reference to a bath compounded from a concentrate containing phosphoric acid, mono-ammonium phosphate, zinc chloride and zinc nitrate in the proportions stated above, it is to be understood that baths compounded from any of the formulations 40 hereinafter set forth may be employed in similar manner.

#### Example II

It is also possible to adapt conventional zinc dihydrogen 45 phosphate compositions to production of amorphous mixed phosphate coatings by modifying the compositions so that they are equivalent to ionized salt-based baths of phosphoric acid, zinc nitrate and ammonium phosphate. Such modified composition in the form of a concentrate 50 may have the following constituents:

|                                             | Composition, Percent by weight |
|---------------------------------------------|--------------------------------|
| Zinc dihydrogen phosphate concentrate (12%) |                                |
| Zn, 48% Po <sub>4</sub> )                   | 68.0                           |
| Zinc chloride                               | 6.0                            |
| Hydrochloric acid (37%, 22° Bé.)            | 8.0                            |
| Ammonium nitrate                            | 13.5                           |
| Water                                       | 4.5                            |
|                                             | 100.0                          |

This composition is prepared by dissolving anhydrous zinc chloride in the zinc dihydrogen phosphate concentrate. The ammonium nitrate is dissolved in the water and hydrochloric acid and the resulting solution is added to the concentrate containing the zinc chloride. The resulting composition is then chemically identical with the concentrate in Example I but is more dilute.

A more concentrated solution can be obtained by first warming the zinc dihydrogen phosphate solution, adding the hydrochloric acid thereto, and then dissolving the ammonium nitrate in the warm solution without additional water, and with the zinc chloride added as the final step. Similar results can be obtained by employing nitric acid and ammonium chloride to convert the zinc chloride, zinc phosphate solution to the desired chemical composition and it will be obvious that other chemicals may be utilized for this. A modifying metal nitrate such as calcium nitrate, lithium nitrate and the like as listed in Example I is added to this bath after the other ingredients in at least the aforesaid minimum or threshold concentrations so as to provide a micro-crystalline phosphate coating.

### Example III

The first two examples described formulations for providing an amorphous mixed phosphate coating and disclosed the addition of the nitrate of the modifier metal after the other ingredients, provided in the form of a concentrate, had been diluted to substantially bath strength. However, the nitrate of the modifier metal may also be included as part of the concentrate as, for example:

| Chemical                                    | Units, Formula Weight×No. of Mols | Composition, Percent By Weight |
|---------------------------------------------|-----------------------------------|--------------------------------|
| Phosphoric acid $H_3PO_4$ .....             | 96×0.08                           | 7.8                            |
| Mono-ammonium phosphate $NH_4H_2PO_4$ ..... | 115×0.10                          | 11.5                           |
| Zinc chloride $ZnCl_2$ .....                | 136×0.04                          | 5.5                            |
| Zinc nitrate $Zn(NO_3)_2$ .....             | 189×0.06                          | 11.3                           |
| Calcium nitrate $Ca(NO_3)_2$ .....          | 164×0.14                          | 23.0                           |
| Water to dissolve.....                      |                                   | 40.9                           |
|                                             |                                   | 100.0                          |

This concentrate was diluted to a 4% by volume solution, heated to 190-200° F. and was employed as a coating bath for a wide variety of articles including ferrous automobile wheels and rims, low carbon steel tubing prior to drawing, and die-cast zinc hardware. The bath was maintained at a 20 to 30 point strength (or total acid strength) and had a ratio of total to free acid of between 5-10 to 1. Coatings were produced by immersion of the cleaned work in the bath for a period of 4 to 8 minutes and the coatings so obtained were smooth and uniform, with no crystal structure visible under magnification of 100 diameters. These coatings provided an excellent undercoat for paint as well as affording excellent corrosion resistance when covered with lanolin or a wax type rust inhibiting film. In addition, the coatings also evidenced ability to hold a lubricant for subsequent drawing operations.

The proportions of the ingredients of this concentrate may be varied from the presently preferred values stated above within the following ranges:

| Chemical                                    | Units, Formula Weight×No. of Mols | Composition, Percent by Weight |
|---------------------------------------------|-----------------------------------|--------------------------------|
| Phosphoric acid $H_3PO_4$ .....             | 98×(0.04 to .12)                  | 5.0 to 15.0                    |
| Mono-ammonium phosphate $NH_4H_2PO_4$ ..... | 115×(0.02 to .15)                 | 7.0 to 15.0                    |
| Zinc chloride $ZnCl_2$ .....                | 136×(0.01 to .10)                 | 1.0 to 10.0                    |
| Zinc nitrate $Zn(NO_3)_2$ .....             | 189×(0.02 to .10)                 | 0.5 to 15.0                    |
| Calcium nitrate $Ca(NO_3)_2$ .....          | 164×(0.10 to .50)                 | 12.0 to 48.0                   |

Amorphous zinc phosphate coatings can be obtained by spraying as well as by immersion, the chief difference in

the baths being that the spray must have a lower free acid and can be run at a lower strength. For example, a spray bath needs only 10 to 20 total points but should have an acid ratio of from 15 to 50. The required low free acid may be initially obtained by neutralizing the free acid with zinc dust, zinc oxide or calcium carbonate, sodium or ammonium hydroxides or by sodium nitrite. The resulting acid balance does not change rapidly since the baths do not hydrolyze under continuous heating. Moreover, the crystal inhibiting salts are neutral and exert a buffer action to stabilize the bath against free acid formation. However, the low permissible free acid in spray formulations limits the solubility of the coating salts in the concentrate so that it is advisable to package the low acid zinc phosphate separately from the nitrate or other salt of lithium, beryllium, magnesium, calcium, strontium, cadmium, or barium to avoid recrystallization of the ingredients.

### Example IV

An effective spray bath for producing an amorphous coating can be prepared from the following:

| Chemical                                                                 | Units, Formula Weight×No. of Mols | Composition, Percent by Weight |
|--------------------------------------------------------------------------|-----------------------------------|--------------------------------|
| A. Zinc salt concentrate:<br>Mono-ammonium phosphate $NH_4H_2PO_4$ ..... | 115×0.125                         | 14.4                           |
| Zinc dihydrogen phosphate $Zn(H_2PO_4)_2$ .....                          | 261×0.125                         | 32.6                           |
| Ammonium chloride $NH_4Cl$ .....                                         | 53×0.125                          | 6.6                            |
| Water to dissolve.....                                                   |                                   | 46.4                           |
|                                                                          |                                   | 100.0                          |
| B. Calcium Nitrate:<br>$Ca(NO_3)_2 \cdot 4H_2O$ .....                    | 236×0.20                          | 47.2                           |
| Water to provide 66% calcium nitrate solution.....                       |                                   | 23.6                           |
|                                                                          |                                   | 70.8                           |

The bath was prepared by mixing the above ingredients together and with water in quantities such that the resulting solution contains 1.5% by volume of the composition designated A above and 1% by volume of that designated B, the free acid being reduced by zinc dust in an amount in the order of 0.1% by weight of the zinc concentrate A. The resulting bath analyzed 20 points, with a ratio of 25 total acid to 1 of free acid, and was maintained at a temperature in the order of 160-170° F. At this strength and temperature an amorphous mixed phosphate coating of 200 mg. per sq. ft. was produced on ferrous metals by spraying them for 1 minute. The bath was found by analysis to contain 2 grams per liter of zinc, 6 grams per liter of phosphate and 12 grams per liter of calcium nitrate, and was held at this level by a constant drip addition of both the concentrates designated A and B.

The proportions of the ingredients in the concentrate employed in compounding this bath may be varied from the presently preferred values stated above within the following ranges:

| Chemical                                        | Units, Formula Weight×No. of Mols |
|-------------------------------------------------|-----------------------------------|
| Mono-ammonium phosphate $NH_4H_2PO_4$ .....     | 115×(0.05-0.20)                   |
| Zinc dihydrogen phosphate $Zn(H_2PO_4)_2$ ..... | 261×(0.05-0.25)                   |
| Ammonium chloride $NH_4Cl$ .....                | 53×(0.05-0.15)                    |
| Calcium nitrate $Ca(NO_3)_2 \cdot 4H_2O$ .....  | 236×(0.10-0.50)                   |

Instead of packaging the zinc salts as one concentrate and the calcium nitrate as the second concentrate, both the zinc and calcium salts can be put together as one concentrate and the phosphate supplied separately as another concentrate.

As mentioned heretofore, conventional zinc phosphate baths can be converted to provide an amorphous coating

of a mixed phosphate and an example of how this may be accomplished has been given above. In general, it has been found that for best results the nitrate or other soluble salt of lithium, beryllium, magnesium, calcium, strontium, cadmium or barium should be employed in an amount at least equimolar with the zinc phosphate and that an accelerating agent be used. The preferred accelerating agents are the neutralizing oxidizers such as sodium nitrite, calcium hypochlorite and barium nitrate which decompose in the bath to leave a neutralizing cation in solution after the gaseous oxidant is released.

The above specific examples have employed a nitrate of lithium, beryllium, magnesium, calcium, strontium, cadmium or barium as an inhibitor of crystal formation in zinc phosphating formulations and other ingredients have been included to facilitate the coating formation. These are not, however, inflexible requirements since any zinc phosphate coating bath can be made to produce an amorphous mixed phosphate coating bath by employing a salt of one of the above mentioned coating crystal inhibitor metals in the presence of a nitrate. Hence, it is not necessary that the nitrate of the crystal inhibitor metal be used since a different soluble nitrate, as for example sodium nitrate, may be added if nitrate is not already present. Moreover, the nitrate may be supplied in combination with the zinc and/or the inhibitor metal may even be employed as the phosphate thereof.

Thus, satisfactory amorphous coatings were provided by immersion of ferrous articles in baths from the following concentrates. The baths were operated at temperatures near boiling and with a total acid of 25 points and a free acid of 4:

*Example V*

| Chemical                                                         | Units, Formula<br>Weight $\times$ No. of<br>Mols | Concentration,<br>Percent By<br>Weight |
|------------------------------------------------------------------|--------------------------------------------------|----------------------------------------|
| Concentrate A:                                                   |                                                  |                                        |
| Calcium monobasic phosphate $\text{Ca}(\text{H}_2\text{PO}_4)_2$ | $252 \times 0.10$                                | 25.2                                   |
| Phosphoric acid $\text{H}_3\text{PO}_4$                          | $98 \times 0.06$                                 | 6.6                                    |
| Zinc nitrate $\text{Zn}(\text{NO}_3)_2$                          | $297 \times 0.05$                                | 14.8                                   |
| Water to dissolve                                                |                                                  | 53.4                                   |
|                                                                  |                                                  | 100.0                                  |
| Concentrate B:                                                   |                                                  |                                        |
| Calcium chloride $\text{CaCl}_2$                                 | $110 \times 0.15$                                | 16.5                                   |
| Mono-ammonium phosphate<br>$\text{NH}_4\text{H}_2\text{PO}_4$    | $115 \times 0.15$                                | 17.2                                   |
| Zinc nitrate $\text{Zn}(\text{NO}_3)_2$                          | $297 \times 0.07$                                | 22.2                                   |
| Phosphoric acid $\text{H}_3\text{PO}_4$                          | $98 \times 0.07$                                 | 6.9                                    |
| Water to dissolve                                                |                                                  | 37.2                                   |
|                                                                  |                                                  | 100.0                                  |

The bath, Concentrate B, operated satisfactorily but was improved by adding ammonium nitrate in the order of 8% of the concentrate.

The amount of the salt of the modifier metal, namely, lithium, beryllium, magnesium, calcium, strontium, cadmium or barium, which may be employed in baths formulated in accordance with this invention is not limited to the minimum or threshold values specified but may be increased when additional buffering action of the added base and the accelerating action of high nitrate concentration are desirable. For example, in formulations for use in spray type baths, the quantity of modifier salt may be two or three times the threshold value set forth. In such a case and in other relatively high concentrations of the modifier metal, the latter may be in greater concentration than the zinc in the modified bath and hence adjustments must be made in the bath to maintain balance and avoid sludge. This may be effected by adding phosphoric acid in amounts to provide a pH of from 2 to 3. Excessive nitrate in the bath may be avoided by employing the chlorides of zinc, lithium, beryllium, magnesium, calcium, strontium, cadmium or barium as part of the bath components rather than supplying all of these elements in the form of the nitrate.

The following example illustrates still another bath for forming integral amorphous phosphate coatings.

*Example VI*

- 5 A predominately iron phosphate film can be formed on ferrous stock by dipping it in solution of a diacidic phosphate such as sodium dihydrogen phosphate, potassium dihydrogen phosphate, ammonium dihydrogen phosphate, magnesium dihydrogen phosphate or calcium dihydrogen phosphate accelerated with an oxidizing or reducing agent. Suitable oxidizing agents are sodium chlorate, sodium nitrite, sodium nitrate, hydrogen peroxide, potassium persulfate, picric acid, quinone, and various other chlorates, bromates, and iodates. Likewise, suitable reducing agents are sodium sulfite, sodium thiosulfate, and sodium phosphite. Thus a concentrate may be made of the following composition:

|                              | Parts |
|------------------------------|-------|
| $(\text{NH}_4)_2\text{PO}_4$ | 75    |
| $\text{CaCl}_2$              | 11    |
| $\text{H}_2\text{O}$         | 14    |

This is made up 5 percent by volume into an iron phosphating solution. This bath could be accelerated by bubbling in gaseous nitrosyl chloride or by adding aqueous nitrobetaine, or  $\text{NOCl}$  amine complexes or Roussin's salts which are nitroso complexes of iron and sulfur. These are further described on page 678 of the Fritz Ephraim's Inorganic Chemistry, 4th ed. (1943). This is an improvement to the Glen L. Williams Patent No. 1,514,494 which disclosed phosphating solutions containing an unstable mixture of aqua regia and Steffan's sugar beet waste as accelerators. Zinc dihydrogen phosphate or manganese dihydrogen phosphate can be used in place of the diacidic phosphate such as mono-ammonium phosphate in the foregoing example if a heavier mixed zinc or manganese and iron phosphate is required.

The following example illustrates a bath which provides an amorphous manganese phosphate coating.

*Example VII*

A concentrate having the following composition by weight was used as a concentration of 5% by weight:

|                      | Percent |
|----------------------|---------|
| Manganese chloride   | 18      |
| Calcium nitrate      | 42      |
| Monosodium phosphate | 26      |
| Diglycolic acid      | 14      |

The bath was broken in to contain some iron and ferrous articles were immersed therein at about 165° F. 50 until a gunmetal grey non-crystalline coating was formed. This coating provided excellent properties as an undercoating to the adhesive bonding of rubber to the coated metal surface. In Example VII, diglycolic acid may be substituted by other reducing agents such as 55 sugars or glycols, aldehydes and sulfites. These reducing agents when used with the nitrate form a reduced nitrate (or nitrite) accelerator.

In a like manner when manganese and iron phosphate coatings are desired, the manganese and iron ions may 60 replace the zinc ions in the foregoing examples by using such chemicals as manganese dihydrogen phosphate, mono-ammonium phosphate, manganese chloride, and ammonium chloride.

The present invention also relates to a method of 65 forming a dry mixture of chemicals used for phosphate coating baths which produce both crystalline and micro-crystalline coatings on the work. In accordance with this aspect of the invention, zinc nitrate is coated with zinc oxide before mixing with other coating materials of 70 which calcium chloride, sodium acid phosphate and an acid selected from a member of the group consisting of diglycolic acid and sulfamic acid are preferably used to make a phosphate coating bath.

The zinc nitrate crystals are coated with a crusty, 75 cement-like coating of zinc oxide by mixing about 5

pounds of zinc oxide with about 30 to 200 pounds of zinc nitrate or about 2 to 16% by weight of the zinc oxide based on the weight of the zinc nitrate. The adherent zinc oxide coating prevents any appreciable deliquescent action by the zinc nitrate and any subsequent reaction of the nitrate with a hydrogen atom of the acid or the sodium acid phosphate to form nitric acid. Also urea may be used with the zinc oxide at a rate of about 1 to 6% by weight of the zinc nitrate in order to prevent a reduction of the nitrate and to react with any nitrous acid fumes that might be formed by thermal decomposition of the nitrate.

The calcium chloride crystals, also being deliquescent are prevented from forming a hydrate by coating the crystals with about 2 to 16 percent by weight calcium phosphate. Calcium oxide may also be used as the coating material, although results are not as good since the calcium oxide itself tends to pick up some water and the sulfamic acid tends to dissolve the oxide if it becomes moist.

The zinc nitrate and calcium chloride are preferably dehydrated before applying their respective coatings. Generally, zinc nitrate or calcium chloride crystals that have been exposed to the atmosphere should be dried so as to eliminate any substantial amount of water of crystallization.

The sulfamic acid or diglycolic acid is preferably coated with starch so as to isolate the acid from the zinc oxide coating and the like which would tend to dissolve in the acid in the presence of substantial amounts of moisture. The amount of starch used as the coating agent is generally about 5 to 15 percent by weight of the acid. The sulfamic acid is added to provide acidity to the bath as well as to reduce the amount of sludge formed. The sulfamic acid is reactive with nitrous acid and, when free to react, tends to scavenge any nitrous acid fumes that might be formed from the decomposition of nitrates.

For best results, the materials should be intimately mixed by suitable means such as ribbon-type mixers and packaged in metal or fiber drums which may be lined with polyethylene or other plastic film.

The dry mixture may be accurately weighed and easily dumped or otherwise placed in a tank of water. Generally the dry mixture is used at a rate of about 1/2 to 20 percent by weight of the total bath although the best coating results are obtained at a concentration of about 4 to 8 parts by weight.

The following dry mixtures are illustrative of the present invention:

| Parts by weight                                                                 |       |
|---------------------------------------------------------------------------------|-------|
| Zinc nitrate (coated with from about 2 to 16% by weight of zinc oxide)          | 20-40 |
| Monosodium phosphate                                                            | 30-50 |
| Calcium chloride (coated with from 2-16 percent by weight of calcium phosphate) | 10-30 |
| Sulfamic acid (coated with from 5-15% by weight of starch)                      | 2-20  |

The following example is for the purpose of illustration and is not intended to limit the invention in any way:

#### Example VIII

An intimate, dry mixture of ingredients was made according to the recipe that follows:

| Parts by weight                                                                               |    |
|-----------------------------------------------------------------------------------------------|----|
| Zinc nitrate (coated with zinc oxide at a ratio of 5 lbs. zinc oxide to 150 lb. zinc nitrate) | 30 |
| Calcium chloride (coated with calcium phosphate by using 10% by weight of calcium phosphate)  | 20 |
| Mono sodium phosphate                                                                         | 40 |
| Sulfamic acid (coated by mixing with 10% by weight of starch)                                 | 10 |

Fifty pounds of the above mixture was dumped into

100 gallons of water and stirred to form an aqueous solution. The bath was maintained at 165° F. and iron ions were supplied to the bath by scrap iron. Freshly pickled cold rolled steel panels were immersed therein for 10 minutes. The surfaces of the steel panels were observed to have a fine, smooth, amorphous-like phosphate coating.

As previously noted and hereinafter more fully described, different percentages of the different ingredients described in Example VIII, such as zinc nitrate, may be used to obtain benefits of the present invention. Calcium chloride may be substituted for by zinc chloride, which may be given a protective coating of zinc oxide, calcium oxide or calcium phosphate. Calcium nitrate may be used in place of the zinc nitrate and other suitable means of supplying the Ca, NO<sub>3</sub>, PO<sub>4</sub>, Zn and Cl ions may be used as long as the ratios of Ca ion to Zn ion, Ca ion to NO<sub>3</sub> ion and NO<sub>3</sub> ion to PO<sub>4</sub> ion are maintained within the previously disclosed ranges.

#### Example IX

A powder spray bath was made according to the following formula:

| Ingredients:                                                                                       | Parts by weight |
|----------------------------------------------------------------------------------------------------|-----------------|
| Zinc nitrate (coated with 10% zinc oxide by weight)                                                | 33              |
| Sodium acid phosphate (coated with 5% starch by weight)                                            | 34              |
| Calcium nitrate (coated with 5% calcium acid phosphate powder, known as dry sugar acid, by weight) | 33              |

Twenty pounds of this powder is dumped into 100 gallons of water and stirred to form an aqueous solution. 10 pounds of calcium nitrate is added at the start of the operation to insure an amorphous coating. The bath is maintained at 170° F. This solution is sprayed on clean steel panels by conventional spray equipment to form a smooth, amorphous coating. If desirable, the iron of the bath can be controlled by addition of sodium nitrite in amounts of 4 to 12 oz. per 100 gallons of bath. The bath is maintained at 8-12 points by addition as required.

When predominantly iron phosphate or manganese phosphate coatings are desired, other ingredients may be used such as ammonium phosphate, ammonium dihydrogen phosphate as previously more fully described.

The baths are also preferably accelerated with suitable oxidizing agents (such as sodium chlorate, sodium nitrate or sodium nitrite) or reducing agents (such as sodium sulfite or sodium thio-sulfate).

While sulfamic acid is preferred as the solid acid of the dry mixture, diglycolic acid or carbamide phosphoric acid may be used although an excessive sludging action of the bath results from their use. Normally aqueous solutions of acids such as glycolic acid may be used, but in this case the dry material is mixed without the liquid acid. The acid is then added to the water when the bath is made up with the dry mixture.

This application is a continuation in part of my pending application Serial No. 274,839 filed March 4, 1952, now abandoned, which is a continuation-in-part of application Serial No. 193,290 filed October 31, 1950, now Reissue Patent No. 24,017, formerly U.S. Patent No. 2,588,234.

It is to be understood in accordance with the provisions of the patent statutes, the particular form of product shown and described and the particular procedure set forth are presented for purposes of explanation and illustration and that various modifications of said product and procedure can be made without departing from my invention.

Having described my invention, what I claim is:

1. A phosphate coating bath make-up compound in powder form comprising 20 to 40 parts of zinc nitrate

particles having a zinc oxide coating thereon, 2 to 20 parts of acid particles selected from a member of the group consisting of diglycolic acid and sulfamic acid with a coating of starch on its particles, 30 to 50 parts of mono-basic sodium phosphate, 10 to 30 parts of calcium chloride having a coating of calcium phosphate powder on its particles so that said composition can be mixed with water to make a non-sludging phosphate coating bath.

2. A method of making a phosphate coating bath make-up compound in powder form comprising the steps of coating zinc nitrate with zinc oxide by mixing about 5 pounds of zinc oxide with about 30 to 200 pounds of zinc nitrate, coating calcium chloride with calcium phosphate by mixing with the calcium chloride about 2 to 16 percent of its weight of calcium phosphate, and mixing said coated zinc nitrate and calcium chloride with relatively dry sulfamic acid and mono-basic sodium phosphate to form a stable dry powdery mixture.

## References Cited in the file of this patent

## UNITED STATES PATENTS

|           |            |               |
|-----------|------------|---------------|
| 1,291,352 | Allen      | Jan. 14, 1919 |
| 2,121,574 | Romig      | June 21, 1938 |
| 2,312,855 | Thompson   | Mar. 2, 1943  |
| 2,499,261 | Rosenbloom | Feb. 28, 1950 |
| 2,500,915 | Tanner     | Mar. 14, 1950 |
| 2,528,787 | Roland     | Nov. 7, 1950  |
| 2,540,314 | Amundsen   | Feb. 6, 1951  |
| 2,588,234 | Henricks   | Mar. 4, 1952  |

## FOREIGN PATENTS

|         |               |               |
|---------|---------------|---------------|
| 440,215 | Great Britain | Dec. 23, 1935 |
| 517,049 | Great Britain | Jan. 18, 1940 |
| 648,888 | Great Britain | Jan. 17, 1951 |
| 310,756 | Germany       | July 1, 1922  |